

## UNITED STATES PATENT OFFICE

2,012,686

PROCESS FOR FIRE-PROOFING  
CELLULOSIC MATERIALSMartin Leatherman, Hyattsville, Md., dedicated  
to the free use of the Public of the United  
States of AmericaNo Drawing. Application May 2, 1934,  
Serial No. 723,546

3 Claims. (Cl. 91—68)

(Granted under the act of March 3, 1883, as  
amended April 30, 1928; 370 O. G. 757)

This application is in part a continuance of my application Serial Number 711,727, filed February 17, 1934.

This application is made under the act of 5 March 3, 1883, as amended by the act of April 30, 1928, and the invention herein described, if patented, may be manufactured and used by or for the Government for governmental purposes without the payment to me of any royalty thereon.

10 I hereby dedicate the invention herein described to the free use of the Public in the territory of the United States of America to take effect upon the granting of a patent to me.

15 This invention relates to an improvement in the fireproofing of cellulosic materials which also largely prevents the out-of-door deterioration of cellulosic fabrics arising from the effects of certain general classes of treating materials, when acted upon by sunlight.

20 It is well known that hydrated stannic oxide prevents flaming of cellulosic materials when properly placed therein. However, it has never been established as to why or how stannic oxide inhibits flaming of cellulosic fabrics when the said 25 fabrics are exposed to an igniting flame. I have discovered the mechanism involved in this said flameproofing process and in order to make these specifications as complete as possible I will briefly describe my discoveries and also the manner in which these discoveries were authenticated.

30 The three lines of investigation which I followed all tended to prove that stannic oxide flameproofs cellulose by setting up a catalytic dehydration of the cellulose under the influence of heat. In the first place, when untreated fabric samples and flameproofed fabric samples were 35 respectively heated in tubes at 325° C. in a stream of dry, CO<sub>2</sub>- free air, the exit gases obtained from the flameproofed fabric samples invariably showed much the larger percentage of CO<sub>2</sub>. The samples in all cases were completely ashed before the air flow was stopped. The air and the gases swept out with it were all collected in a large evacuated bottle each time and aliquot samples of the collected gas were analyzed in a modified Orsat apparatus. The larger yield of CO<sub>2</sub> from the treated samples indicated to me that with the treated, flameproofed samples the 40 products formed were largely CO<sub>2</sub> and water, whereas with the untreated samples the carbon was evolved as a constituent of volatile combustible compounds such as acetone, hydrocarbons, etc.

45 50 55 In the second phase of my investigations the

carefully dried fabric samples were heated in tubes in a stream of dried oxygen-free nitrogen, the tubes being immersed in a molten metal bath at 325° C. for 240 seconds. The tarry matter was filtered out of the exit gases and the evolved moisture was collected and weighed. The percentage of water evolved, based on the net weight of the fabric, was always much greater in the case of the samples treated with stannic oxide.

5 10 15 The third line of study was undertaken to establish beyond any doubt that the stannic oxide effects its flameproofing action by splitting the cellulose into carbon and water. Treated and untreated samples were heated at 325° C. in tubes in a stream of dried oxygen-free nitrogen until most of the matter volatile at that temperature was driven off, the heating being continued the same length of time in all cases. The container tubes were then connected with an absorption train and the fabric residues were completely 20 25 30 burned in a stream of oxygen. In this way the carbon in the residues was determined as carbon dioxide. Based on the net weight of carbon in the original cellulose of the fabric samples, the percentage of carbon in the residues from the destructive distillation of the treated fabric was 35 nearly twice as great as in the identically obtained residues from the untreated fabric.

Thus it was definitely proved that stannic oxide flameproofs cellulose by catalytically splitting the cellulose carbohydrate into carbon and water and thereby preventing the formation of combustible gases. It now became possible to improve the action of stannic oxide by applying known principles of catalysis. In the first place, it has been shown by others that alkali acts as a catalyst poison. Therefore, if it were possible to precipitate stannic oxide in the cotton fabric under more acid conditions a more pronounced flameproofing effect should be produced. The Perkin method Patent No. 856,906 of using fairly dilute ammonium sulfate solutions to decompose the sodium stannate on the fabric precipitates the stannic oxide under alkaline conditions because of the ammonia evolved.

40 45 50 55 If, for example, instead of using ammonium sulfate as the precipitant for sodium stannate, ferric sulfate or chloride is used, three effects are obtained. In the first place a solution of ferric sulfate or of ferric chloride is acid in reaction, as is ammonium sulfate, because of hydrolysis.

The reaction between sodium stannate and the ferric salt, if an excess of the latter is used, leaves the solution from which the stannic oxide is deposited still acid, unlike ammonium sulfate, and

this lessens the quantity of alkali which can be absorbed by the freshly precipitated, gel-like stannic oxide. In the second place, ferric oxide is precipitated in intimate contact with the stannic oxide and thereby exerts catalytic promoter effects. Many other oxides exert similar effects. In the third place, and most important, the iron oxide colors the fabric and this coloring exerts a preservative action on the fabric. This is true of other colored oxides such as those of chromium, manganese, copper, cobalt, nickel, etc. Stannic oxide alone in fabric accelerates deterioration of cotton fabric in sunlight.

The desirable catalytic action of stannic and other oxides in flameproofing of cellulose is accompanied by a most undesirable action. These oxides are also catalysts for carbon combustion and after the dehydration mechanism liberates the carbon the oxide facilitates its combustion. Consequently flameproofed fabrics glow vigorously even though they do not flame. For this reason, to produce a fully fireproofed fabric, after flameproofing with metallic oxides, it is necessary to use a supporting agent. From the standpoint of weather-resistance there is only one type of material which will suffice. This type of material is represented by chlorinated organic substances of various kinds. It is known to use the chlorinated vinyl resins in combination with tin oxide, but, while this treatment effectively fireproofs cotton, it is impracticable because both stannic oxide and chlorinated vinyl resin act very destructively on the fabric so that the fabric lasts only a short time. However, I have discovered that this destructive action is prevented by the presence of a coloring material.

In the past, the chlorinated resinous materials have all been objectionable because of cost or undesirable physical or chemical properties. I have found that certain cheap petroleum derivatives can be chlorinated to give materials which are very well suited as glowproofing agents for use in connection with oxide mixtures in cellulose fabrics for exposure to weather. The glowproofing effect results from the evolution of hydrogen chloride at elevated temperatures. The chlorinated product must not decompose spontaneously when properly protected, that is, by a coloring material, and it must evolve hydrogen chloride within a definite temperature range. I have discovered that highly chlorinated paraffin wax answers these requirements but does not have the desired physical properties, that is, it stiffens the fabric too much. If, before chlorination, I mix with the paraffin approximately its own weight of certain light bodied partially unsaturated liquid paraffin oils of low lubricating power, such as are used by filling stations for flushing crank cases, I can introduce a higher percentage of chlorine and still obtain a less plastic product which does not unduly stiffen the fabric but results in a flexible, soft, fire-proofed material which is also highly water proofed. I prefer to have in the finished chlorinated material fifty to seventy per cent of chlorine based on the total weight of product but the percentage of chlorine may, within the spirit of my invention, be less or more than this.

It is well known that tin is a rare metal and that its cost must progressively increase. One of the further merits of my invention lies in the fact that by using promoter oxides, a part of the tin necessary for flameproofing may be replaced with cheaper metal oxides. An additional merit of my invention lies in the possibility of assisting, with-

out deleterious results, the flameproofing effect of the oxides by using the above-mentioned resinous chlorinated petroleum derivatives, which besides glowproofing the fabric, markedly assist in fireproofing it.

A typical procedure which I may follow in producing a weather-resistant fireproofing treatment in cellulose fabrics is as follows: if the fabric is unbleached and water-resistant it is first soaked in a solution of a wetting agent of either the sulfonated type or of the sulfate ester type for about five minutes, such as a one per cent aqueous solution of a metallic salt of a sulfate ester of an aliphatic alcohol, then squeezed out and rinsed thoroughly in water for about five minutes, after which it is again squeezed out and immersed in sodium stannate solution for about twenty minutes. When bleached and absorbent fabric is being treated the wetting agent treatment is unnecessary. The sodium stannate solution contains about twenty parts or less of alpha sodium stannate in one hundred parts of water. The fabric is dried by any suitable means after soaking in the stannate solution and then put into a twenty per cent aqueous solution of ferric sulfate. This produces a tan colored fabric. Instead of iron salts, such salts as chromium sulfate, manganous sulfate, vanadium chloride, titanous sulfate, or any salt of a strong mineral acid with a weakly base-forming metal, the hydroxide of which is water-insoluble, may be used. Where the precipitating salt does not leave a colored precipitate, as in the case of titanium or vanadium salts, it is necessary to use a previously colored fabric or to introduce a pigment later, preferably with the resin treatment. It may also be desirable to mix enough iron or chromium salt with the titanium salt solution to produce a colored precipitate in the fabric.

After the precipitation of the stannate, the fabric is squeezed and immersed in aqueous or gaseous ammonia to precipitate the balance of the iron or other metal which may have been used. This additional amount of colored oxide obtained by the ammonia precipitation is of great value in that it gives a deeper color than that provided when the colored metallic salts are washed out, and this deeper color is very effective in further preserving the fabric against deterioration. When the ammonia precipitation is used, less washing of the fabric is required, in fact, where the sodium and ammonium salts are not objectionable the fabric need not be washed at all. However, ammonium salts tend to deteriorate the fabric in time and it will usually be desirable to wash them out. After drying, the fabric is ready for the treatment with the glowproofing agent.

I have found that certain of the chlorinated diphenyls act as excellent plasticizers in connection with my chlorinated petroleum derivatives, and, in fact, in connection with other chlorinated resinous materials. The best chlorinated diphenyl derivative is one which exists as a moderately viscous liquid but I may use a chlorinated diphenyl derivative which is less viscous or one which is solid. All of the derivatives obtained by chlorinating diphenyl are of value. These materials by themselves do not materially assist in preventing flaming in cellulosic materials but when used as I describe they appear to slightly assist the flame- and glow-proofing action of the material which they serve to plasticize.

The percentage of chlorinated diphenyl to be required as a plasticizing material will depend upon the physical properties of the said chlori-

nated diphenyl as well as upon other factors. I may use as little as fifteen parts of chlorinated diphenyl to eighty-five parts of chlorinated petroleum derivatives and I may use enough to equal 5 the weight of the chlorinated petroleum derivatives employed. In general the total mixture impregnated into the fabric will not exceed thirty per cent of the total weight of the treated fabric, including precipitated oxides. For most purposes, twenty per cent of the total weight of the finished fireproofed fabric will be sufficient.

As a plasticizing agent there may be substituted in the place of chlorinated diphenyls specified above, other plasticizing materials such as tri- 15 phenyl phosphate, tricresyl phosphate or dibutyl phthalate.

For purposes of clarity I will define the terms "flameproofed" and "fireproofed" as they are used 20 in these specifications. "Flameproofed" fabric denotes fabric which has been treated with metallic oxides and has thereby been made resistant to flaming but has not been made glow-resistant; in fact, the glow tendency will usually be considerably increased in flameproofed fabrics. "Fireproofed" fabric denotes fabric which 25 will not propagate flame and which will not propagate flameless combustion or glowing beyond the charred portion of the fabric which has been subjected to an igniting flame.

Having made a full disclosure of the function 30 of the glowproofing and assisting agent I will now give specific examples of compositions which are suitable for my purpose.

As a typical composition of the glowproofing 35 resin I may use 75 parts of chlorinated petroleum products, preferably a chlorinated mixture of paraffin wax and low-viscosity, partially unsaturated, petroleum oils, said chlorinated mixture to contain approximately sixty per cent of chlorine based on total weight, and 25 parts of chlorinated diphenyl. For my purpose I will ordinarily use as 40 a plasticizer a chlorinated diphenyl which has a viscosity similar to that of heavy molasses. However, I do not restrict myself because I can use the chlorinated petroleum derivatives without any plasticizer at all or I can use chlorinated diphenyls of a wide range of physical properties mixed with the chlorinated petroleum derivatives in widely varying proportions.

In coating or impregnating the flame-proofed 45 fabric with the chlorinated resinous glowproofing and assisting agent no definite solution concentrations can be specified because the proper and desired concentration will vary with the solvent employed, the pressure applied in squeezing out 50 excess solution and with the percentage which it is desired to leave in the fabric. For a given concentration of solution, a high-volatile solvent like carbon tetrachloride will leave a higher percentage of resin in the fabric than will low-volatile solvents such as mineral spirit thinners. Also if the fabric is to be treated by dipping, the 55 concentration will be different than if the resin solution is applied by brushing.

The proportions of the respective ingredients 60 present in the finished fireproofed fabric may be varied considerably. For example, if the percentage of flameproofing oxides is increased, the percentage of glowproofing resin can be decreased to a certain point. Also the glowproofing resin solution may be made the vehicle for a pigment, and a paint may thereby be prepared which is especially useful in preparing striped awnings or in home treating of canvas on farms or else-

where. As pigment any earthy material such as ochre, sienna, umber, etc., or any colored metallic oxide may be used.

In the treatment as outlined in these specifications there is no water-soluble constituent which 5 can be leached out by rain and the pigmenting material stabilizes the chlorinated resinous constituent. The fabric retains its fireproof characteristics and does not rapidly lose its tensile strength as it will do when no pigment is present. 10

The petroleum hydrocarbons furnish a cheap 15 source of raw material for chlorination and the finished chlorinated product is cheap enough to be used in low priced fabrics.

Having fully disclosed my invention, I claim: 18

1. The process of fire-proofing and preserving 20 cellulosic materials and fabrics which comprises immersing the fabric until thoroughly saturated in a one per cent aqueous solution of a metallic salt of a sulfate ester of an aliphatic alcohol, rinsing the cellulosic material thoroughly in water, pressing out as much of the water as possible; then impregnating the cellulosic material with sodium stannate, drying, and then immersing the dried cellulosic material in a water solution of a salt of a strong mineral acid with a weakly base-forming metal, the hydroxide of which is water-insoluble, then with only light squeezing immersing the wet cellulosic material 25 in an ammonia solution, then washing the material in water to remove soluble salts, drying the material, impregnating the material with a chlorinated mixture of paraffin wax and low-viscosity, partially unsaturated petroleum oil 30 plasticized with chlorinated diphenyl derivatives 35 and containing coloring materials.

2. The process of fire-proofing and preserving 40 cellulose materials and fabrics which comprises immersing the fabric until thoroughly saturated in a one per cent solution of a metallic salt of a sulfate ester of an aliphatic alcohol, rinsing the cellulosic material thoroughly in water, pressing out as much of the water as possible; then impregnating the cellulosic material with sodium stannate, drying, and then immersing the dried 45 cellulosic material in an aqueous solution of ferric sulphate, then with light squeezing immersing the wet cellulosic material in an ammonia solution, then washing the cellulosic material in water to remove soluble salts, drying the cellulosic material and impregnating it with a chlorinated mixture of paraffin wax and low-viscosity, partially unsaturated petroleum oil containing chlorinated diphenyl derivatives.

3. The process of fire-proofing and preserving 55 cellulosic materials and fabrics which comprises immersing the fabric until thoroughly saturated in a one per cent aqueous solution of a metallic salt of a sulfate ester of an aliphatic alcohol, rinsing the cellulosic material thoroughly in 60 water, pressing out as much of the water as possible; then impregnating the cellulosic material with sodium stannate, drying, and then immersing the dried cellulosic material in a water solution of a salt of a strong mineral acid with a 65 weakly base-forming metal, the hydroxide of which is water-soluble and colored, then washing the material in water to remove acid residues, drying the material and impregnating the material with a chlorinated mixture of paraffin wax 70 and low-viscosity, partially unsaturated petroleum oil.

MARTIN LEATHERMAN.

**CERTIFICATE OF CORRECTION.**

Patent No. 2,012,686.

August 27, 1935.

**MARTIN LEATHERMAN.**

It is hereby certified that error appears in the printed specification of the above numbered patent requiring correction as follows: Page 3, second column, line 67, claim 3, for "water-soluble" read water-insoluble; and that the said Letters Patent should be read with this correction therein that the same may conform to the record of the case in the Patent Office.

Signed and sealed the 5th day of November, A. D. 1935.

Leslie Frazer

(Seal)

Acting Commissioner of Patents.